



US005316687A

## United States Patent [19]

Bloink et al.

[11] Patent Number: 5,316,687

[45] Date of Patent: May 31, 1994

[54] ELECTRORHEOLOGICAL COMPOSITIONS INCLUDING  $A_{1+x}Zr_2Si_xP_{3-x}O_{12}$ 

[75] Inventors: Raymond L. Bloink, Swartz Creek; Bob R. Powell, Birmingham, both of Mich.

[73] Assignee: General Motors Corporation, Detroit, Mich.

[21] Appl. No.: 702,973

[22] Filed: May 20, 1991

[51] Int. Cl.<sup>5</sup> ..... C10M 171/00; C10M 169/04

[52] U.S. Cl. ..... 252/71; 252/73;

252/74; 252/75; 252/572

[58] Field of Search ..... 252/71, 73, 74, 572,  
252/75

## [56] References Cited

## U.S. PATENT DOCUMENTS

|           |         |                 |       |             |
|-----------|---------|-----------------|-------|-------------|
| 2,417,850 | 3/1947  | Winslow         | ..... | 175/320     |
| 3,839,252 | 10/1974 | Bosso et al.    | ..... | 260/29.2 EP |
| 4,645,614 | 2/1987  | Goossens et al. | ..... | 252/75      |
| 4,687,589 | 8/1987  | Block et al.    | ..... | 252/73      |
| 4,744,914 | 5/1988  | Filisko et al.  | ..... | 252/74      |
| 4,772,407 | 9/1988  | Carlson         | ..... | 252/74      |
| 4,879,056 | 11/1989 | Filisko et al.  | ..... | 252/74      |

## FOREIGN PATENT DOCUMENTS

|            |         |                    |   |
|------------|---------|--------------------|---|
| 0311984    | 4/1989  | European Pat. Off. | . |
| 0361931    | 4/1990  | European Pat. Off. | . |
| 0387857    | 9/1990  | European Pat. Off. | . |
| WO82/04442 | 12/1982 | PCT Int'l Appl.    | . |
| 1570234    | 6/1980  | United Kingdom     | . |

## OTHER PUBLICATIONS

Block et al, "Electro-rheology", J. Phys. D: Appl. Phys., 21(12), 1661-77, 1988.

Heng, "Crystal Structures and Crystal Chemistry in the System  $Na_{1+x}Ar_2Si_xP_{3-x}O_{12}$ ", Mat. Res. Bull. vol. 11, pp. 173, 182, 1976.Goodenough et al, "Fast  $Na^+$ -Ion Transport in Skeleton Structures", Mat. Res. Bull. vol. 11, pp. 203-220, 1976.Hong et al, "High  $Na^+$ -Ion Conductivity in  $Na_5YSi_4O_{12}$ ", Mat. Res. Bull. vol. 13, pp. 757-761, 1978. Pergamon Press, Inc. Printed in the U.S.

Clearfield et al, "New Crystalline Phases of Zirconium

Phosphate Processing Ion-Exchange Properties", J. inorg. nucl. Chem. 1968, vol. 30, pp. 2249-2258. Pergamon Press. Printed in Great Britain.

Maazaz et al, "Sur Une Nouvelle Famille De Conducteurs Cationiques A Structure Feuilletee De Formule  $K_x(L_{x/2}Sn_{1-x/2})O_2(L=Mg, Ca, Zn, x \leq 1)$ ", Mat. Res. Bull. vol. 14, pp. 193-199, 1979. Printed in the USA. Copyright (c) Pergamon Press Ltd.Alberti et al, "All Solid State Hydrogen Sensors Based on Pellicular  $\alpha$ -Zirconium Phosphate as a Protonic Conductor", Solid State Ionics, vol. 35, No. 1, 2 Jul.-/Aug. 1989, pp. 153-156.Shannon et al, "Ionic Conductivity in  $Na_5YSiO_{12}$ -Type Silicates", Inorganic Chemistry, vol. 17, No. 4, 1978, pp. 958-964.Miller et al, "A Prepilot Process for the Fabrication of Polycrystalline  $\beta$ -Alumina Electrolyte Tubing", Ceramic Bulletin, vol. 58, No. 5 (1979), pp. 522-526.

Hooper et al, "Ionic Conductivity of Pure and Doped

(List continued on next page.)

Primary Examiner—Christine Skane  
Attorney, Agent, or Firm—Cary W. Brooks

[57]

## ABSTRACT

Disclosed are electrorheological fluids having ceramic particles of high ion conductivity and a nonconducting or dielectric fluid. The high ion conductive particle may be a material having the formula  $A_{1+x}Zr_2Si_xP_{3-x}O_{12}$ , where A is a monovalent ion, such as a material comprising at least one selected from the group consisting of Li, Na, K, Ag and Cu; and x ranges from 0 to 3. The liquid phase may include a silicone fluid or mineral oil. In the case of a mineral oil, the oil may also include an amine-terminated polyester to improve stability of the fluid.

7 Claims, 1 Drawing Sheet



## OTHER PUBLICATIONS

$\text{Na}_3\text{PO}_4$ ", Journal of Solid State Chemistry 214, 265-275 (1978).

West, "Ionic Conductivity of Oxides Based on  $\text{Li}_4\text{SiO}_4$ ", Journal of Applied Electrochemistry 3 (1973), pp. 327-335.

Hu et al, "Ionic Conductivity of Lithium Phosphate-Doped Lithium Orthosilicate", Mat. Res. Bull. vol. 11, pp. 1227-1230, 1976. Pergamon Press, Inc. Printed in the U.S.

Hu et al, "Ionic Conductivity of Lithium Or-

thosilicate-Lithium Phosphate Solid Solutions", J. Electrochem. Soc.: Solid-State Science and Technology, vol. 124, No. 8, Aug. 1977, pp. 1240-1242.

Delmas et al, "Ionic Conductivity in Sheet Oxides", Copyright 1979 by Elsevier North Holland, Inc. Vashishta, Mundy, Shenoy, eds. Fast Ion Transport in Solids, pp. 451-454.

Delmas, "Sur De Nouveaux Conducteurs Ioniques A Structure Lamellaire", Mat. Res. Bull. vol. 11, pp. 1081-1086, 1976. Pergamon Press, Inc. Printed in the U.S.



FIG. 1

**ELECTRORHEOLOGICAL COMPOSITIONS  
INCLUDING  $A_{1+x}Zr_2Si_xP_{3-x}O_{12}$**

**FIELD OF THE INVENTION**

The present invention relates to fluid compositions which demonstrate significant changes in their flow properties in the presence of an electric field.

**BACKGROUND OF THE INVENTION**

Electrorheology is a phenomenon in which the rheology of a fluid is modified by the imposition of an electric field. Fluids which exhibit significant changes in their properties of flow in the presence of an electric field have been known for several decades. The phenomenon of electrorheology was reported by W. M. Winslow, U.S. Pat. No. 2,417,850, in 1947. Winslow demonstrated that certain suspensions of solids in liquids show large, reversible electrorheological effects. In the absence of an electric field, electrorheological fluids generally exhibit Newtonian behavior. That is, the applied force per unit area, known as shear stress, is directly proportional to the shear rate, i.e., change in velocity per unit thickness. When an electric field is applied, a yield stress appears and no shearing takes place until the shear stress exceeds a yield value which generally rises with increasing electric field strength. This phenomenon can appear as an increase in viscosity of up to several orders of magnitude. The response time to electric fields is on the order of milliseconds. This rapid response, characteristic of electrorheological fluids makes them attractive to use as elements in mechanical devices.

A complete understanding of the mechanisms through which electrorheological fluids exhibit their particular behavior has eluded workers in the art. Many have speculated on the mechanisms giving rise to the behavior characteristics of electrorheological fluids.

A first theory is that the applied electric field restricts the freedom of particles to rotate, thus changing their bulk behavior.

A second theory ascribes the change in properties to the filament-like aggregates which form along the lines of the applied electric field. The theory proposes that this "induced fibrillation" results from small, lateral migrations of particles to regions of high field intensity between gaps of incomplete chains of particles, followed by mutual attraction of these particles. Criticism of a simple fibrillation theory has been made on the grounds that the electrorheological effect is much too rapid for such extensive structure formation to occur; workers in the art have observed a time scale for fibrillation of approximately 20 seconds, which is vastly in excess of the time scale for rheological response of electrorheological fluids. On the other hand, response times for fibrillation on the order of milliseconds have been observed.

A third theory refers to an "electric double layer" in which the effect is explained by hypothesizing that the application of an electric field causes ionic species adsorbed upon the discrete phase particles to move, relative to the particles, in the direction along the field toward the electrode having a charge opposite that of the mobile ions in the adsorbed layer. The resulting charge separation and polarization could lead to "dipole" interactions and fibrillation.

Yet another theory proposes that the electric field drives water to the surface of discrete phase particles through a process of electro-osmosis. The resulting

water film on the particles then acts as a glue which holds particles together. If correct, then a possible sequence of events in fibrillation would be: ionic migration, subsequent electro-osmosis of moisture to one pole of the particle (presumably the cationic region) and bridging via this surface supply of water. However, the advent of anhydrous electrorheological fluids means that water-bridging is not an essential mechanism and may indeed not be operative at all.

Despite the numerous theories and speculations, it is generally agreed that the initial step in development of electrorheological behavior involves polarization under the influence of an electric field. This then induces some form of interaction between particles or between particles and the impressed electric or shear fields which results in the rheological manifestations of the effect. See Carlson, U.S. Pat. No. 4,772,407; and Block et al "Electro-Rheology", IEEE Symposium, London, 1985. Despite this one generally accepted mechanism, the development of suitable electrorheological fluids and methods of improving the same remains largely unpredictable.

The potential usefulness of electrorheological fluids in automotive applications, such as vibration damping, shock absorbers, or torque transfer, stems from their ability to increase, by orders of magnitude, their viscosity upon application of an electric field. This increase can be achieved with very fast (on the order of milliseconds) response times and with minimal power requirements.

Although ER-fluids have been formulated and investigated since the early 1940's, basic limitations have prevented their utilization in practical devices. The most restrictive requirements are (1) that the suspensions be stable over time, i.e., that the solid particles either remain suspended in the liquid or be readily redispersed if sedimentation occurs and (2) service and durability of the suspensions can be achieved outside the temperature range of 0-100°C. This latter requirement is particularly restrictive in that most fluid compositions require water as an ER "activator" so that in completely nonaqueous systems the ER-effect is entirely absent or so small that it is not effectively useful.

An object of this invention is to formulate a stable, substantially water-free, or nonaqueous ER-fluid with improved properties.

**SUMMARY OF THE INVENTION**

This invention generally includes electrorheological fluids having ceramic particles of high ion conductivity and a nonconducting or dielectric fluid. The high ion conductive particle may be a material having the formula  $A_{1+x}Zr_2Si_xP_{3-x}O_{12}$ , where A is a monovalent ion, such as a material comprising at least one selected from the group consisting of Li, Na, K, Ag and Cu; and x ranges from about 0 to about 3. These ceramic particles of high ion conductivity eliminate the need for water in the electrorheological fluids. It is believed that the structure of the material is such that ions are mobile within and/or on the surface of the particle. These mobile ions produce a charge separation (dipoles) on the surface of the particle in the presence of an electric field. Under the influence of an electric field, the dipoles of the particles could interact resulting in chains of particles extending between electrodes and which require additional energy to shear. Such chains produce a higher viscosity in the electrorheological fluid. Where

the invention comprises anhydrous fluids, the elimination of the requirement for water in the electrorheological fluid expands the operating temperature outside of 0-100°C.

These and other objects, features and advantages of this invention will be apparent from the following detailed description, appended drawings and claims.

#### BRIEF DESCRIPTION OF THE DRAWINGS

FIG. 1 is a graphic illustration of the viscosity of an electrorheological fluid according to the present invention both in the presence and absence of an electric field.

#### DETAILED DESCRIPTION OF THE INVENTION

The solid phase of an electrorheological fluid according to the present invention comprises a high ion conductive material including a material having the formula  $A_{1+x}Zr_2Si_xP_{3-x}O_{12}$ , where A is a monovalent ion, such as at least one selected from the group consisting of Li, Na, K, Ag, and Cu; and where x ranges from about 0 to about 3. Solid phase materials may be prepared by conventional techniques known to those skilled in the art. A suitable method of preparing a solid phase is described in Hong, "Crystal Structures and Crystal Chemistry in the System  $Na_{1+x}Zr_2Si_xP_{3-x}O_{12}$ ", Materials Research Bulletin, Vol. 11, pages 173-182, (1976), which is hereby incorporated by reference.

Preferably, the materials of the solid phase are in the form of particles such as spheres, cubes, whiskers, or platelets. Preferably, the particles are equiaxed. The particles have an effective length or diameter ranging from about 0.1 to about 75 micrometers. The particles may be present in the fluid in an amount ranging from about 5 to about 50, and preferably about 15 to about 30 percent by volume of the composition.

Preferably, the material of the solid phase is dried at a temperature ranging from about 200°C. to about 600°C., preferably 400°C. to about 600°C. and most preferably 600°C., which is sufficient to remove any residual water on the solid phase but not alter the structure of the solid. The particles are referred to as being substantially free of water. The term "substantially free of water" means less than 0.5 percent by weight water adhering (i.e., absorbed or adsorbed) to the particles. Preferably, the amount of water adhering to the particles is less than that required for the water to be an "activator" of electrorheological response. That is, the amount of water adhering to the particles of the solid phase is not sufficient to create water bridges between particles under the influence of an electric field. The drying of the particles is carried out under low vacuum at a constant pressure. Preferably the drying is at a pressure ranging from about 300 to about 50 mTorr, preferably 200 to about 50 mTorr and most preferably at 50 mTorr. The resultant, dry particles are then dispersed in a liquid phase.

Suitable liquid phase materials include any nonconductive substance that exists in a liquid state under the conditions which a fluid using it would be employed. Any nonconducting fluid in which particles could be dispersed would be suitable. A preferred fluid is silicone fluid. Other suitable liquid phase materials are disclosed in Block et al, "Electro-Rheology", IEEE Symposium, London, 1985, which is hereby incorporated by reference. A suitable silicone fluid is commercially available

from Union Carbide under the trade name SILICONE FLUID L45/10 TM.

The stability of the electrorheological fluid may be improved by adding a dispersant or stabilizer to the liquid phase. When the liquid is a mineral oil, a preferred stabilizer is an amine-terminated polyester, such as SOLSPERSE 17000 TM available from ICI Americas. An electrorheological fluid was prepared as described above wherein the solid phase consisted of a material having the composition  $Na_{3.3}Zr_2Si_{2.3}P_{0.7}O_{12}$  and the liquid phase consisted of mineral oil. As can be seen in FIG. 1, in the presence of an electric field the fluid exhibited a dramatic increase in viscosity compared to the fluid in the absence of electric field.

The various embodiments may be combined and varied in a manner within the ordinary skill of persons in the art to practice the invention and to achieve various results as desired.

Where particular aspects of the present invention are defined herein in terms of ranges, it is intended that the invention includes the entire range so defined, and any sub-range or multiple sub-ranges within the broad range. By way of example, where the invention is described as comprising one to about 100 percent by weight component A, it is intended to convey the invention as including about five to about 25 percent by weight component A, and about 50 to about 75 percent by weight component A. Likewise, where the present invention has been described herein as including  $A_{1-100}B_{1-50}$ , it is intended to convey the invention as  $A_{1-60}B_{1-20}$ ,  $A_{60-100}B_{25-50}$  and  $A_{43}B_{37}$ .

The embodiments of the invention in which an exclusive property or privilege is claimed are defined as follows:

1. An electrorheological composition comprising:  
a solid phase present in an amount ranging from about 5 to about 50 percent by volume of said composition comprising a material having the formula  $A_{1+x}Zr_2Si_xP_{3-x}O_{12}$ , where A is a monovalent ion, and X ranges from about 0 to about 3; and  
a liquid phase comprising a dielectric fluid, said composition being substantially free of water and effective to produce an electrorheological response in the presence of an electric field.

2. An electrorheological composition as set forth in claim 1 wherein A is selected from the group consisting of Li, K, Na, Ag and Cu.

3. An electrorheological composition as set forth in claim 1 wherein said solid phase comprises particles having a size ranging from about 1 to about 5 micrometers in length.

4. An electrorheological composition as set forth in claim 1 wherein said solid phase is about 5 to about 30 volume percent of said electrorheological composition.

5. An electrorheological composition as set forth in claim 1 wherein said liquid phase comprises silicone fluid.

6. A method of producing an electrorheological response in a composition comprising:  
adding particles having the formula  $A_{1+x}Zr_2Si_xP_{3-x}O_{12}$  where A is a monovalent ion and x ranges from about 0 to about 3, to a dielectric fluid to from an electrorheological composition in an amount ranging from about 5 to about 50 percent by volume of said composition, said composition being substantially free of water; and

applying an electric field to said composition so that the viscosity of said composition increases.

7. An electrorheological composition comprising a solid phase comprising  $Na_{3.3}Zr_2Si_{2.3}P_{0.7}O_{12}$  present in an amount ranging from about 5 to about 50 percent by 5

volume of said composition, and a liquid phase comprising a dielectric fluid, said composition being substantially free of water and effective to produce an electrorheological response in the presence of an electric field.

\* \* \* \* \*

10

15

20

25

30

35

40

45

50

55

60

65

**Disclaimer**

5,316,687—Raymond L. Bloink, Swartz Creed; Bob R. Powell, Birmingham, both of Mich. ELECTORHEOLOGICAL COMPOSITONS INCLUDING  $A_{1+x}ZR_2Si_xP_{3-x}O_{12}$ . Patent dated May 31, 1994. Disclaimer filed June 19, 1997, by the assignee, General Motors Corp.

Hereby enters this disclaimer to claims 1-7 of said patent.